

Dec. 8, 1964

R. KRETSCH

3,159,964

PROCESS FOR WORKING UP STRETCHED FILAMENTS OF AROMATIC  
POLYESTERS OF HIGH MOLECULAR WEIGHT

Filed Jan. 30, 1962

2 Sheets-Sheet 1

FIG. 1



FIG. 2



INVENTOR  
ROSL KRETSCH

BY Connolly and Dut  
his ATTORNEYS

Dec. 8, 1964

R. KRETSCH

3,159,964

PROCESS FOR WORKING UP STRETCHED FILAMENTS OF AROMATIC  
POLYESTERS OF HIGH MOLECULAR WEIGHT

Filed Jan. 30, 1962

2 Sheets-Sheet 2

FIG. 3



INVENTOR  
ROSL KRETSCH

BY *Connolly and Stauff*  
for ATTORNEYS

1

3,159,964

## PROCESS FOR WORKING UP STRETCHED FILAMENTS OF AROMATIC POLYESTERS OF HIGH MOLECULAR WEIGHT

Rosl Kretsch, Bobingen, near Augsburg, Germany, assignor to Farbwerke Hoechst Aktiengesellschaft vormals Meister Lucius &amp; Brüning, Frankfurt am Main, Germany, a corporation of Germany

Filed Jan. 30, 1962, Ser. No. 169,782

Claims priority, application Germany, Feb. 11, 1961, F 33,189; Mar. 17, 1961, F 33,434  
11 Claims. (Cl. 57—157)

The present invention relates to a process and an apparatus for working up stretched filaments of aromatic polyesters of high molecular weight.

Filaments of aromatic polyesters of high molecular weight have hitherto been worked up in discontinuous manner by twisting the stretched filaments and winding them up on a bobbin, the core of which consists of an elastic wire structure. The wound-up filaments are then subjected on the bobbin to a prolonged steam treatment, whereby shrinkage occurs and the filaments are simultaneously set. After said heat-setting the filaments are wound up on saleable bobbins.

The present invention provides a process and an apparatus which enable stretched polyester filaments to be worked up into a finished saleable form in one continuous operation. According to the process of the invention the stretched filament is twisted and the twisted filament is passed through a solution, dispersion, or emulsion of at least one substance boiling within the range of 120° C. to 350° C. and then fed to two rollers, which serve as fixed points and rotate at different speeds and around each of which the filament is passed several times, the first of the rollers being heated. Between these rollers, the filament is heated on all sides uniformly to a temperature within the range of 220° C. to 350° C., preferably 250° C. to 280° C., for 0.1 to 5 seconds, advantageously 0.2 to 1 second, and allowed to undergo an adjustable shrinkage of 5 to 35%, preferably 10-25%. Thereupon the filament is stretched again by the same degree or a higher degree or a smaller degree and wound up on a bobbin. In general the after-stretching is carried out in a manner such that the finished filament possesses the most favorable shrinkage on boiling and thermo-shrinkage required for the further processing in the weaving and knitting mill, so that a setting of the filament can be dispensed with. The term "shrinkage on boiling" indicates the degree of shrinkage in percent a filament undergoes when dipped into boiling water. By the term "thermo-shrinkage" there is to be understood the degree of shrinkage a filament undergoes when kept for a few seconds in hot air of 200° C. If the filament is after-stretched by the same degree or a higher degree, it is of advantage to treat it with steam or dry hot air.

FIG. 1 is a diagrammatic view of one embodiment according to the invention.

FIG. 2 is a diagrammatic view of another embodiment according to the invention.

FIG. 3 is a diagrammatic view of still another embodiment according to the invention.

The process of the invention can be carried out as follows: (cf. FIGURE 1 of the accompanying drawings).

The stretched filament of linear aromatic polyesters is wound up on a cop which is placed on a spindle 1 rotating at a high speed and the filament is drawn off upwardly whereby it is twisted. It is then conducted over a thread guide 2 and a guide roll 3 into a container 4 which is charged with a treating liquid. The filament is then dried on heated roller 5 and passed through heater 7 having a temperature within the range of 220° C. to 350° C.

2

Between rollers 5 and 8, which serve as fixed points and around which the filament is wrapped several times, the filament is allowed to shrink by 5 to 35%. The filament is then fed to a further roller 10 having a higher speed than roller 8 so that between roller 8 and roller 10 the filament is stretched by 5-35%. Subsequently the filament is wound up on bobbin 14.

A further mode of execution of the process of the invention is illustrated with reference to FIGURE 2.

- 10 The filament is twisted and passed through the treating liquid as described above. Subsequently, it is dried on heated roller 5, passed through heating channel 7 (temperature 220° C.-350° C.) and fed to roller 8 rotating at a lower speed. Between roller 5 and roller 8 the filament is allowed to shrink by the desired degree. The filament is then passed to a third roller 10' which is mounted as stepped roller on roller 5. Stepped roller 10' rotates at a higher speed than roller 8 so that the filament is stretched between roller 8 and the stepped roller to a degree which is smaller than that of the previous shrinkage. After stretching, the filament is wound up on bobbin 14 via guide roller 12 and changeable thread guide 13. Drying roller 5 has preferably a temperature within the range of 50° C. to 120° C.
- 20 In the process of the invention the filament is passed through a solution, dispersion or emulsion of at least one substance boiling within the range of 120° C. and 350° C. which can be removed later on by washing or has the character of a preparation and is therefore not detrimental if it remains behind on the filament. The chemical nature of the substance is only of minor importance. Decisive are its physical properties. A wide variety of substances may therefore be used for carrying out the process of the invention. The substances should boil at a temperature in the range of 120° C. to 350° C.; at room temperature they may be fluid, syrupy, pasty or may form films. Crystalline substances of low molecular weight are less suitable for use since they deposit on the rollers. A well suitable substance is, for example, sorbitol, a sugar alcohol which is syrupy at room temperature. Besides there may be used other mono- or polyhydric high-boiling alcohols, such as glycerol, lauryl alcohols, glycols, and polyglycols. Furthermore, there may advantageously be used substances containing one or several reactive groups, for example hydroxyl or carboxyl groups, as well as substances that are free from reactive groups and swell the polyester filament, for example high-boiling esters, high-boiling ethers or aromatic high-boiling hydrocarbons such as diphenyl. Still further, there are suitable for wetting the filaments higher molecular mono- or di-carboxylic acids as far as they do not decompose at a temperature above 200° C., and the esters thereof, for example terephthalic acid di-butyl ester or tricresyl phosphate; high-boiling phenols, amines and amino-alcohols, for example ethyl-amines, diethanolamines and triethanolamines, as far as they do not produce yellowing of the filaments on heating; polymeric compounds, for example polyacrylic acid and the esters thereof, polymethylacrylic acid, polyvinyl alcohols and esters of polyvinyl alcohols. The solutions, emulsions or dispersions are advantageously prepared with the use of water or an organic solvent boiling below 100° C.
- 30 In the process of the invention the filament is passed through a solution, dispersion or emulsion of at least one substance boiling within the range of 120° C. and 350° C. which can be removed later on by washing or has the character of a preparation and is therefore not detrimental if it remains behind on the filament. The chemical nature of the substance is only of minor importance. Decisive are its physical properties. A wide variety of substances may therefore be used for carrying out the process of the invention. The substances should boil at a temperature in the range of 120° C. to 350° C.; at room temperature they may be fluid, syrupy, pasty or may form films. Crystalline substances of low molecular weight are less suitable for use since they deposit on the rollers. A well suitable substance is, for example, sorbitol, a sugar alcohol which is syrupy at room temperature. Besides there may be used other mono- or polyhydric high-boiling alcohols, such as glycerol, lauryl alcohols, glycols, and polyglycols. Furthermore, there may advantageously be used substances containing one or several reactive groups, for example hydroxyl or carboxyl groups, as well as substances that are free from reactive groups and swell the polyester filament, for example high-boiling esters, high-boiling ethers or aromatic high-boiling hydrocarbons such as diphenyl. Still further, there are suitable for wetting the filaments higher molecular mono- or di-carboxylic acids as far as they do not decompose at a temperature above 200° C., and the esters thereof, for example terephthalic acid di-butyl ester or tricresyl phosphate; high-boiling phenols, amines and amino-alcohols, for example ethyl-amines, diethanolamines and triethanolamines, as far as they do not produce yellowing of the filaments on heating; polymeric compounds, for example polyacrylic acid and the esters thereof, polymethylacrylic acid, polyvinyl alcohols and esters of polyvinyl alcohols. The solutions, emulsions or dispersions are advantageously prepared with the use of water or an organic solvent boiling below 100° C.
- 40 In the process of the invention the filament is passed through a solution, dispersion or emulsion of at least one substance boiling within the range of 120° C. and 350° C. which can be removed later on by washing or has the character of a preparation and is therefore not detrimental if it remains behind on the filament. The chemical nature of the substance is only of minor importance. Decisive are its physical properties. A wide variety of substances may therefore be used for carrying out the process of the invention. The substances should boil at a temperature in the range of 120° C. to 350° C.; at room temperature they may be fluid, syrupy, pasty or may form films. Crystalline substances of low molecular weight are less suitable for use since they deposit on the rollers. A well suitable substance is, for example, sorbitol, a sugar alcohol which is syrupy at room temperature. Besides there may be used other mono- or polyhydric high-boiling alcohols, such as glycerol, lauryl alcohols, glycols, and polyglycols. Furthermore, there may advantageously be used substances containing one or several reactive groups, for example hydroxyl or carboxyl groups, as well as substances that are free from reactive groups and swell the polyester filament, for example high-boiling esters, high-boiling ethers or aromatic high-boiling hydrocarbons such as diphenyl. Still further, there are suitable for wetting the filaments higher molecular mono- or di-carboxylic acids as far as they do not decompose at a temperature above 200° C., and the esters thereof, for example terephthalic acid di-butyl ester or tricresyl phosphate; high-boiling phenols, amines and amino-alcohols, for example ethyl-amines, diethanolamines and triethanolamines, as far as they do not produce yellowing of the filaments on heating; polymeric compounds, for example polyacrylic acid and the esters thereof, polymethylacrylic acid, polyvinyl alcohols and esters of polyvinyl alcohols. The solutions, emulsions or dispersions are advantageously prepared with the use of water or an organic solvent boiling below 100° C.
- 50 In the process of the invention the filament is passed through a solution, dispersion or emulsion of at least one substance boiling within the range of 120° C. and 350° C. which can be removed later on by washing or has the character of a preparation and is therefore not detrimental if it remains behind on the filament. The chemical nature of the substance is only of minor importance. Decisive are its physical properties. A wide variety of substances may therefore be used for carrying out the process of the invention. The substances should boil at a temperature in the range of 120° C. to 350° C.; at room temperature they may be fluid, syrupy, pasty or may form films. Crystalline substances of low molecular weight are less suitable for use since they deposit on the rollers. A well suitable substance is, for example, sorbitol, a sugar alcohol which is syrupy at room temperature. Besides there may be used other mono- or polyhydric high-boiling alcohols, such as glycerol, lauryl alcohols, glycols, and polyglycols. Furthermore, there may advantageously be used substances containing one or several reactive groups, for example hydroxyl or carboxyl groups, as well as substances that are free from reactive groups and swell the polyester filament, for example high-boiling esters, high-boiling ethers or aromatic high-boiling hydrocarbons such as diphenyl. Still further, there are suitable for wetting the filaments higher molecular mono- or di-carboxylic acids as far as they do not decompose at a temperature above 200° C., and the esters thereof, for example terephthalic acid di-butyl ester or tricresyl phosphate; high-boiling phenols, amines and amino-alcohols, for example ethyl-amines, diethanolamines and triethanolamines, as far as they do not produce yellowing of the filaments on heating; polymeric compounds, for example polyacrylic acid and the esters thereof, polymethylacrylic acid, polyvinyl alcohols and esters of polyvinyl alcohols. The solutions, emulsions or dispersions are advantageously prepared with the use of water or an organic solvent boiling below 100° C.
- 60 In the process of the invention the filament is passed through a solution, dispersion or emulsion of at least one substance boiling within the range of 120° C. and 350° C. which can be removed later on by washing or has the character of a preparation and is therefore not detrimental if it remains behind on the filament. The chemical nature of the substance is only of minor importance. Decisive are its physical properties. A wide variety of substances may therefore be used for carrying out the process of the invention. The substances should boil at a temperature in the range of 120° C. to 350° C.; at room temperature they may be fluid, syrupy, pasty or may form films. Crystalline substances of low molecular weight are less suitable for use since they deposit on the rollers. A well suitable substance is, for example, sorbitol, a sugar alcohol which is syrupy at room temperature. Besides there may be used other mono- or polyhydric high-boiling alcohols, such as glycerol, lauryl alcohols, glycols, and polyglycols. Furthermore, there may advantageously be used substances containing one or several reactive groups, for example hydroxyl or carboxyl groups, as well as substances that are free from reactive groups and swell the polyester filament, for example high-boiling esters, high-boiling ethers or aromatic high-boiling hydrocarbons such as diphenyl. Still further, there are suitable for wetting the filaments higher molecular mono- or di-carboxylic acids as far as they do not decompose at a temperature above 200° C., and the esters thereof, for example terephthalic acid di-butyl ester or tricresyl phosphate; high-boiling phenols, amines and amino-alcohols, for example ethyl-amines, diethanolamines and triethanolamines, as far as they do not produce yellowing of the filaments on heating; polymeric compounds, for example polyacrylic acid and the esters thereof, polymethylacrylic acid, polyvinyl alcohols and esters of polyvinyl alcohols. The solutions, emulsions or dispersions are advantageously prepared with the use of water or an organic solvent boiling below 100° C.

65

70

75

80

85

90

95



the degree of whiteness of the filaments is improved.

3  
It is also possible to apply a sizing agent to the filaments by adding such sizing agent to the treating bath. Excellent sized filaments are obtained, for example, with the use of emulsions of acid polyacrylic acid esters.

When filaments shall be prepared which have an especially good dyeability and an improved handle and gloss, it is of advantage to use, instead of filaments having a round cross section, filaments having a larger surface area, such as filaments the cross section of which has the shape of a triangle, star, dumb bell and the like. Under the same conditions of treatment, filaments of this kind absorb a larger quantity of dyestuff than filaments having a round cross section so that it is possible to obtain very dark dyeings without the use of carriers.

In special cases it may be advantageous to treat filaments of polyethylene terephthalate having a low viscosity, for example a specific viscosity in the range of 0.450 to 0.700. By specific viscosity there is to be understood the viscosity of a 1% solution of the polyester in a solvent mixture of 60 parts of phenol and 40 parts of tetrachloroethane, determined at 25° C. The dyestuff receptivity of filaments made from a polyester of this kind can be improved under milder conditions, i.e. at lower temperatures and with a lower degree of shrinkage, by the same or a higher percentage than that of filaments made from polyethylene terephthalate having a specific viscosity of 0.800.

According to a further variant of the process of the present invention the chemical substances which improve the dyestuff receptivity of polyester filaments are applied to the filaments not after the twisting but already together with the spinning preparation. It is recommended to use substances, such as high-boiling esters or hydroxyethylated acids, which are suitable as spinning preparation as well as for improving the dyeability. The spun filaments which have been treated with such a spinning preparation are stretched as usual, twisted on the spindle of the apparatus of the invention, again treated with a solution or emulsion of the same compounds as used as spinning preparation, heated at a temperature of above 220° C. while being allowed to shrink and finally stretched again.

Another variant of the process of the invention consists in allowing the filament of linear aromatic polyesters to shrink in a continuous operation at a temperature in the range of 220° C. to 350° C., after it has been re-stretched, by a degree which is smaller than the degree of the prior re-stretching. The filament is subsequently wound up. By this treatment the filament is set so that a further setting by hot air or steam can be dispensed with. This special embodiment of the invention is further illustrated with the aid of the accompanying FIGURE 3.

A stretched polyester filament is twisted with the aid of twisting spindle 1, passed through thread guide 2 and introduced into treating bath 4 which is charged with a solution, dispersion or emulsion of at least one of the substances listed above. The filament is impregnated with said substances and dried on heated roller 5. The filament is then passed through heating chamber 7 where it is allowed to shrink by 5-35% since roller 8 rotates slower than roller 5 by this degree. The filament travels to roller 10' which is mounted as stepped roller on roller 5. The diameter of stepped roller 10' can be equal to or smaller than that of roller 5. The stepped roller rotates at a higher speed than roller 8 so that the filament is stretched between roller 8 and roller 10' by an adjustable degree. After having been stretched the filament is again passed through a heating channel 12' heated at a temperature in the range of 220° C. to 350° C. It then travels over guide roll 13' and changeable thread guide 14' to winding-up roller 15 having a lower circumferential speed than roller 10' so that on the way between roller 10' and winding-up 15 the filament is again allowed to shrink in heating zone 12' by an adjustable degree. When the two shrinkages are effected at the same temperature, it is possible to use one heating chamber instead of the two heat-

ing chambers 7 and 12' which is then passed twice by the filament.

The filaments treated by the process of the invention are finished and can be well dyed with dispersion dyestuffs. Furthermore, the treated filaments possess good textile properties. It is possible, for example, to adjust their shrinking values as desired, depending on the degree of re-stretching. The high elongation which is undesired for many applications is reduced by the re-stretching.

The following examples serve to illustrate the invention but they are not intended to limit it thereto.

#### Example 1

A stretched filament of polyethylene terephthalate having a titer of 100/50, which was wound up on a cop, was twisted to obtain 350 trs./m. and then passed at room temperature through a bath containing 15% of glycerol dissolved in water. The filament was then fed at a speed of 50 m./minute to a drying roller which was heated to 100° C. and to which belonged an intermediate roller, the filament being wrapped 12 times around said latter roller. The filament then travelled through a heating chamber which was 40 cm. long and heated to 250° C. The filament was then drawn off from the draw roller, around which it was wrapped 12 times, at a speed of 37.5 m./minute so that it was allowed to shrink in the heating chamber by 25%. Subsequently, the filament was passed 12 times around a roller having a speed of 42.5 m./minute and to which belonged an intermediate roller, whereby it was stretched again. After having left said roller the filament was wound up. The twisted filament thus obtained was ready for sale and of very good quality. It had a much better dyeability than comparative filaments made from the same cop which had been separately twisted and heat-set with hot steam.

On dyeing with the bromination product of 1,5-diamino-4,8-dihydroxyanthraquinone the filament absorbed 55.5% of the dyestuff used.

#### Example 2

Stretched filaments of polyethylene terephthalate having a titer of 100/50 were twisted and further treated as described in Example 1. Instead of the glycerol solution of 15% strength in water, there was used a 15% solution of sebacic acid dimethyl ester in ethanol. The drying roller was heated at 80° C. and rotated at a speed of 50 m./minute, while the second roller had a speed of only 35 m./minute. Thus the filament was allowed to shrink by 30% on this distance. The filament was then stretched again by 30% and wound up. After said treatment the filament was heat-set for 20 minutes at 110° C. with steam. The filaments obtained could be well dyed with dispersion dyestuffs. On dyeing as described in Example 1, the filaments absorbed 65.0% of the dyestuff used.

#### Example 3

Stretched filaments of polyethylene terephthalate having a titer of 100/50 were twisted and further treated as described in Example 1. The treating bath consisted of a 15% solution of terephthalic acid dibutyl ester in methanol. The first roller was heated at 80° C. and rotated at a speed of 50 m./minute while the second roller had a speed of 35 m./minute so that the filaments were allowed to shrink by 30%. The third roller rotated at a speed of 40 m./minute whereby the filaments were again stretched. The resulting filaments could be excellently dyed with dispersion dyestuffs. On dyeing as described in Example 1 the filaments absorbed 89.0% of the dyestuff used.

#### Example 4

Stretched filaments of polyethylene terephthalate having a titer of 100/50 were twisted and treated as described in Example 1 with a glycerol solution of 15% strength. The first roller was heated at 100° C. and ro-

tated at a speed of 50 m./minute while the second roller had a speed of 35 m./minute so that the filaments were allowed to shrink by 30%. The heating chamber had a temperature of 250° C. The third roller rotated at a speed of 50 m./minute, whereby the filaments were stretched to their initial length. After said treatment, the filaments were heat-set for 20 minutes with hot dry air having a temperature of 180° C. On dyeing as described in Example 1, the resulting filaments absorbed 53.5% of the dyestuff used.

*Example 5*

Stretched filaments of polyethylene terephthalate having a titer of 100/50 and a specific viscosity of 0.620 were twisted as described in Example 1 and treated with a 15% glycerol solution. The first roller was heated at 100° C. and rotated at a speed of 50 m./minute, the second roller had a speed of 40 m./minute. In the heating chamber heated at 250° C. the filaments were allowed to shrink by 20% and then stretched again. The filaments obtained absorbed 74.0% of the dyestuff used when dyed as described in Example 1.

*Example 6*

Stretched filaments of polyethylene terephthalate having a titer of 75/35 and a star-shaped cross section (5 points) were twisted as described in Example 1 and treated with a glycerol solution. The first roller was heated at 100° C. and rotated at a speed of 50 m./minute, while the second roller had a speed of 35 m./minute so that the filaments could shrink by 30% in the heating chamber having a temperature of 250° C. The third roller had a speed of 40 m./minute whereby the filaments were stretched again. The resulting filaments were distinguished by an excellent dyeability with dispersion dyestuffs. They absorbed 89.5% of the dyestuff used when dyed as described in Example 1. Fabrics made from the filaments had a nice silky gloss.

*Example 7*

Stretched filaments having a titer of 75/35 of polyethylene terephthalate (specific viscosity 0.620), the individual capillaries of which had a cross section in the form of a star with five points, were twisted as described in Example 1 and treated with a 15% glycerol solution. The first roller which was heated at 100° C. rotated at a speed of 40 m./minute and the second roller had a speed of 32 m./minute so that the filament was allowed to shrink by 20% in the heating chamber having a temperature of 250° C. The filaments were then stretched again. The resulting filaments absorbed 74.5% of the dyestuff used when dyed as described in Example 1. Woven or knitted articles made from the filaments possessed a wonderful silky gloss.

*Example 8*

Stretched filaments of polyethylene terephthalate having a titer of 100/50, which on spinning had been treated with a preparation consisting of diethyl sebacate and a condensation product from lauric acid with 7 mols of ethylene oxide, were twisted as described in Example 1 and again treated with an emulsion consisting of 15% of diethyl sebacate and 15% of a condensation product from lauric acid with 7 mols of ethylene oxide. The first roller was heated at 100° C. and rotated at a speed of 50 m./minute while the second roller had a speed of 35 m./minute so that the filament shrunk by 30% in the heating chamber having a temperature of 250° C. The third roller rotated at a speed of 45 m./minute whereby the filaments were stretched again. The filaments obtained showed an excellent receptivity for dispersion dyestuffs. When dyed as described in Example 1 they absorbed 87.0% of the dyestuff used.

*Example 9*

A filament of polyethylene terephthalate having a titer of 100/50 was twisted and then passed through an emulsion consisting of 6% of diethyl sebacate, 6% of a condensation product from oleyl alcohol with 5 mols of ethylene oxide and 3% of a condensation product from lauric acid with 7 mols of ethylene oxide in water. The filament was dried on a roller heated at 100° C. around which the filament was wrapped 12 times. The roller had a speed of 50 m./minute. The filament was then passed through a heating chamber 45 cm. long which had a temperature of 250° C. and subsequently wrapped 12 times around a second heated roller rotating at a speed of 35 m./minute so that on the way through the heating chamber between the two rollers the filament was allowed to shrink by 30%. The filament was then reconducted to a third roller mounted as stepped roller on the first roller, heated at 100° C. and rotating at a speed of 50 m./minute. Thus the filament was stretched by the degree it previously shrunk. It was then passed a second time through the heating chamber having a temperature of 250° C., and wound up. The winding-up device had a speed of 40 m./minute so that the filament was again allowed to shrink by 20%. The filament obtained was heat-set. It shrunk by 2.4% in boiling water and 3.64% in hot air of 200° C. In a dye bath containing as dyestuff 3% of the bromination product of 1,5-diamino - 4,8 - dihydroxyanthraquinone (calculated on the weight of the filament) the filament absorbed, in the absence of a carrier, 79.0% of the dyestuff used.

*Example 10*

A filament of polyethylene terephthalate having a titer of 100/50 was twisted as described in Example 9 and passed through an emulsion consisting of 15% of terephthalic acid dibutyl ester and 7.5% of a condensation product from oleyl alcohol and 5 mols of ethylene oxide in water. The filament was dried, allowed to shrink at 250° C. by 30%, against stretched in the cold by 30%, allowed to shrink a second time at 250° C. by 25% and then wound up. The finished filament was set. It shrunk by 2.3% in boiling water and by 4% in air of 200° C. On dyeing as described in Example 9, the filament absorbed 90% of the dyestuff used.

45 I claim:

1. A process for processing stretched filaments of aromatic polyesters of high molecular weight, which comprises twisting the stretched filaments, passing the twisted filament through a bath consisting of a member selected from the group consisting of a solution, dispersion and an emulsion of at least one substance boiling in the range of 120° C. to 350° C., feeding the filament to two rollers which serve as fixed points and rotate at different speeds, the first one of which is heated, wrapping the filament several times around the rollers and heating it between the rollers uniformly on all sides to a temperature within the range of 220° C. to 350° C. for 0.1 to 5 seconds, simultaneously allowing the filament to undergo an adjustable shrinkage of 5 to 35%, again stretching the filament and winding it up, said steps being carried out in one continuous operation.

2. The process of claim 1, wherein the twisted filament is heated to a temperature within the range of 250° C. to 280° C.

3. The process of claim 1, wherein the filament is allowed to undergo an adjustable shrinkage of 10 to 25%.

4. The process of claim 1, wherein the bath consists of a member selected from the group consisting of a monofunctional reactive compound and a polyfunctional reactive compound.

5. The process of claim 1, wherein at least one dispersion dyestuff is added to the bath in addition to the reactive compound.

6. The process of claim 1, wherein an optical brightener is added to the bath.

7. The process of claim 1, wherein the optical brightener is a substance corresponding to the formula



8. The process of claim 1, which comprises re-stretching the shrunk filament by the same degree as it shrunk previously and then winding it up. 10

9. The process of claim 1, which comprises re-stretching the shrunk filament by a smaller degree than it previously shrunk and winding it up. 5

10. The process of claim 1, which comprises re-stretch- 15

ing the shrunk filament by a larger degree than it previously shrunk and winding it up.

11. The process of claim 1, which comprises setting the re-stretched filament in a continuous process at a temperature in the range of 220° C. to 350° C. by allowing it to shrink again by a smaller degree than that of the previous re-stretching, and winding it up.

References Cited in the file of this patent

UNITED STATES PATENTS

|           |                |               |
|-----------|----------------|---------------|
| 2,466,808 | Henning et al. | Apr. 12, 1949 |
| 2,768,057 | Friederich     | Oct. 23, 1956 |
| 2,807,863 | Schenker       | Oct. 1, 1957  |
| 2,846,752 | Lessig         | Aug. 12, 1958 |
| 2,932,078 | Wilson         | Apr. 12, 1960 |